

## UNITED STATES PATENT OFFICE.

EUGENE P. SCHOCH, OF AUSTIN, TEXAS.

## DEHYDRATED LIGNITE AND PROCESS OF PRODUCING THE SAME.

No Drawing.

Application filed July 17, 1922. Serial No. 575,656.

*To all whom it may concern:*

Be it known that I, EUGENE P. SCHOCH, a citizen of the United States, residing at Austin, in the county of Travis and State of Texas, have invented certain new and useful Improvements in Dehydrated Lignite and Processes of Producing the Same; and I do hereby declare the following to be a full, clear, and exact description of the invention, such as will enable others skilled in the art to which it appertains to make and use the same.

This invention relates to dehydrated lump lignite and a process of producing the same, and has for its object to provide a procedure which will be comparatively inexpensive to carry out, and more efficient in practice than those heretofore proposed, while at the same time producing a superior product.

With these and other objects in view, the invention consists in the novel steps and combinations of steps constituting the process and in the novel dehydrated lump lignite fuel constituting the product, all as will be more fully hereinafter disclosed and particularly pointed out in the claims.

In order that the precise invention may be the more clearly understood, it is said:

Fresh lignite as obtained in the mines contains say from 25% to 35% of moisture, which it loses when heated at 110° C. to constant weight. Heated above this temperature, to 300° C. it gives up still more moisture, and some carbon dioxide; and heated still higher it begins to yield tar, and combustible gases; the deep-seated decomposition which it then undergoes involves an exothermic reaction so that the heating power of the products when used as a fuel is less than that of the original material and the decomposition thus entails an actual loss of heating power.

When exposed to air, raw lignite gives up a large fraction of its moisture and disintegrates so extensively as to become mostly dust or fine particles. This same disintegration takes place in the fire when lignite is used as a fuel, and hence, unless special grates are provided, much of the lignite drops unburned into the ash pit. When

heated in retorts or dryers to expel the moisture, lignite disintegrates entirely, producing dust or very small fragments.

The large amount of water in lignite and the fact that it disintegrates whenever it loses its water either in storage or during combustion, naturally affects its commercial value greatly, and hence improved processes for making a better form of fuel out of lignite have been and are being actively sought. The only process heretofore known to me or proposed, for producing a better form of lump fuel from lignite consists of retorting the material and briquetting the resulting powder. This requires 10% or more of a first class asphalt, coal tar pitch or other suitable carbonaceous binder, a mixing operation to impregnate the powder with the binder, and then briquetting the material with strong presses. The difficulty of doing this economically and the high cost of the initial installation has retarded capitalists from entering into this business. It results that the proper machinery, as well as the details of the whole process are to-day still in their experimental stages.

I have discovered, on the other hand, that when fresh lump lignite is heated in a still and immersed in thin petroleum oil, such as gas oil or engine distillate, it gives up its moisture without forming any appreciable amount of powder or small fragments. In fact, the original lumps remain intact, although they may have formed some cracks. Most of these cracks are very fine, while large parts of the pieces are entirely free from cracks.

This invention, however, is not limited to the use of the specific oil mentioned for oils having a paraffine base as well as oils having an asphaltic base of all degrees of thickness can be used, but I prefer a thin oil to a thick one for most purposes.

In carrying out this process, I therefore prefer to cover the lignite entirely with oil and to use the lumps as they ordinarily come from the mine, when they range, say, in smallest dimension from 1 inch to 5 inches, and in largest dimensions from 3 to 8 inches. The time required to raise the

temperature of the mixture to 250° C. in the still is about two hours. At the end of that time, no moisture appears to be coming from the still. The oil is then drained 5 out of the still. An examination of this oil-heated lignite shows that all the lumps retain their original form, and although the treated material is brittle, yet most of the pieces are sufficiently firm to be handled 10 without disintegration. As compared with some of the same lignite which is air-dried simultaneously, the oil-dried lignite shows a much smaller number of cracks, which do not gape open as wide as is the case in the 15 air dried lignite. Further, the fragments formed on breaking the oil dried lignite are relatively large, while the air-dried material is cracked so extensively that it separates readily into very small fragments, and even 20 into dust particles.

In order to improve the physical condition of the oil-heated material still further it may be submerged in hot asphaltic oil such as Mexican crude petroleum of about 12° 25 Bé and retained therein at a temperature of 250° to 300° C. for about two hours. The oil is then drained out of the still while it is hot. When this last named procedure is completed, it is found that the lumps have 30 retained so little of this thick oil on the outside as to leave them practically dry, although the material has been so thoroughly permeated with the oil as to be non-brittle, and hence capable of standing a good deal of 35 handling without extensive breaking of the lumps. In fact, it is found that, at most, only the lumps with diameters larger than 3 to 4 inches may break up and that none of the fragments formed are smaller than a 40 pecan nut, while most of them range in size from a hen's egg upward. I prefer to use a thin oil in the first treatment because a thick oil foams when steam is formed in it at or 45 near the boiling point of water, and it probably does not soak into the cracks as readily at a relatively low temperature as a thin oil does.

Upon examination, the final product produced by the two treatments above described 50 gives the following results:

|                             |                 |
|-----------------------------|-----------------|
| Volatile combustible matter | 51.13%          |
| Fixed carbon                | 39.42%          |
| Ash                         | 9.45%           |
| 55 Heating power            | 13,032 B. t. u. |
| Moisture                    | None.           |

The same raw untreated lignite gives the following results:

|                             |                |
|-----------------------------|----------------|
| 60 Moisture                 | 28.15%         |
| Volatile combustible matter | 32.07%         |
| Fixed carbon                | 31.59%         |
| Ash                         | 8.19%          |
| Heating power               | 8,641 B. t. u. |

Assuming that 10% of oil was retained by 65 the treated lignite and that the oil has a heating power of 19,250 B. t. u. per pound, we obtain the following figures by calculation:

|                                                                                                                                                                |                 |
|----------------------------------------------------------------------------------------------------------------------------------------------------------------|-----------------|
| Heat obtained from the 10% oil in 1 lb. of material                                                                                                            | 1.925 B. t. u.  |
| Heat obtained from the 90% lignite in 1 lb. of material                                                                                                        | 11,107 B. t. u. |
| Heating power of 100% of this lignite without oil                                                                                                              | 12,340 B. t. u. |
| Per cent loss of moisture and other non-combustible volatiles from original lignite required to raise its heating power from 8,640 B. t. u. to 12,340 B. t. u. | 30.0%           |
| Per cent of remaining volatile combustible matter in raw lignite                                                                                               | 30.22           |

It should be noticed that in the above operation the lignite was heated much above 110° C. and that a part of the 32.07% volatile combustible matter of the raw lignite was also expelled. That is, we should take 90 from the above 30% loss of moisture and other non-combustibles the moisture content of 28.15% of the raw lignite to get the difference amounting to 1.85% and this difference of 1.85% should be subtracted from the 32.07 in the raw lignite, thus leaving the 30.22% of remaining volatile combustible matter arrived at before.

The latter per cent of volatile combustible matter (30.22) together with that of fixed carbon (31.59) and ash (8.19) in the raw lignite will be larger in the treated lignite by the amount corresponding to the loss of 30.0% volatiles lost minus 10% of oil added, or in other words, the per cents of those ingredients will be increased in the ratio of 70 to 90, and hence become,

|                                          |        |
|------------------------------------------|--------|
| Volatile combustible matter plus 10% oil | 48.90% |
| Fixed carbon                             | 40.60% |
| Ash                                      | 10.50% |

These figures are found to be in part slightly greater and in part slightly smaller than those obtained by examining the treated lignite. Hence, we may consider that 10% of oil is approximately the amount absorbed. Since the material was allowed to absorb and retain all of the oil that it would, we may further look upon the amount of 10% to be the maximum it can take up. This is of importance in comparing the cost of this process of treating lignite with the cost of another process now proposed for the conversion of lignite to an industrially suitable form, namely that of retorting and briquetting. In the latter process, the lignite is retorted to an extent that removes 115 120 125

all the moisture plus some combustible gas and tar, and in this operation the lignite disintegrates practically entirely into a powder or granular mass. This mass must then be mixed with a suitable binder and pressed, with powerful presses, into briquettes of various suitable shapes.

Many binders have been proposed for this purpose, but at present only two kinds seem to be suitable: (a) a thick asphaltic or pitchy residues left and obtained in the distillation of coal tar or of crude petroleum. These residues must be made up of compounds which are stiff and tough when cold, but thin when hot. (b) Starchy or syrupy residues such as are obtained in making sugar (e. g., black strap molasses), and from paper manufacturing ("sulphite pitch"). These binders are soluble in water and hence are less suitable than the class (a) binders.

The better class of binders—those of class (a) must be used in a minimum amount of 10%. Even this amount will not coat every speck of the lignite powder so thoroughly as to prevent the absorption of moisture. Furthermore, the asphalt or pitch must be of high grade, that is, it must become so stiff on cooling as to give the briquettes the proper rigidity.

These extreme and costly requirements, on the other hand, do not need to be met by the thick oil I use to impregnate the lumps of oil-heated lignite. This thick oil serves to make the mass elastic, and while it glues together some of the split-planes, yet the rigidity is maintained by inherent hardness of most of the material and not by the binder. It is surprising that only 10% of oil is absorbed by this lump lignite, even though no attempt is made to press the cracks, etc., close together. But a probable explanation resides in the fact that none of the tar or oily components of the original lignite are destroyed by my oil-heating process, while any process of retorting lignite certainly destroys from 5% to 10% of these components present. My procedure, accordingly, takes advantage of this important fact.

In order to reduce the volatility or flashing of my product to a minimum I remove the lighter oils from the thick oil by bubbling steam through it while the lignite is heated with it. The resulting oil will naturally "glue up" the cracks somewhat firmer than a thinner oil, yet this is not essential to make the material retain its shape while it is handled. The steaming out of the light oil is done only to remove some of the most volatile oil.

From the foregoing, it will now be clear that my process provides a procedure which is comparatively inexpensive and simple to

carry out, while it also produces fuel lignite of a high calorific value in its natural lump form capable of being handled without briquetting. Further, it is found that this oil treated dehydrated lump lignite is not materially affected by repeated wetting and drying in the hot sun. It does not soften in the flame and the lumps do not crack to an objectionable extent while burning, but retain their form until burned to ash. In other words, the finished product simulates the behavior of bituminous coal on burning, except it does not melt and fuse together.

An important feature of the invention resides in the fact that it requires only relatively cheap oils which are plentiful instead of equal amounts of the expensive asphalts now used in briquetting. The bearing of this upon our large undeveloped lignite deposits needs no comment.

The finished product is preferably produced in the lump form above mentioned, but of course it could be as readily produced in a finer or a coarser form, or it could be used as a raw material like finely divided coal for making briquettes, or it could even be mixed with coal. When in the lump form after treatment with a thin oil it has a toughness comparable with charcoal and dark smooth surfaces. After the treatment with a heavy crude oil the toughness is increased and the lumps take on the dark shiny appearance of soft coal. In both cases the product can be readily distinguished from the raw lignite both by its physical appearance and by its toughness.

It is obvious that those skilled in the art may vary the details of the procedure, as well as the form of the finished product without departing from the spirit of the invention, and therefore I do not wish to be limited to the above disclosure except as may be required by the claims.

What is claimed is:

1. The process of treating lignite which comprises heating the same in contact with a hydrocarbon oil to drive off the moisture present, and removing the oil not absorbed by the material, substantially as described.

2. The process of treating lignite which comprises coating the same with a hydrocarbon oil; heating the coated lignite to a temperature sufficient to drive off a substantial portion of the moisture present; and removing any oil not absorbed by the lignite, substantially as described.

3. The process of treating lignite which comprises coating the same in the form of lumps with a hydrocarbon oil; heating the coated lignite to a temperature sufficient to drive off a substantial portion of the moisture present but insufficient to destroy its

lump like form; and removing any oil not absorbed by the lignite, substantially as described.

4. The process of treating lignite which consists in coating lumps of the raw material with a hydrocarbon oil; heating the coated lumps to a temperature sufficient to dehydrate the same; draining off any oil

not absorbed by said lumps; again heating said lignite with a hydrocarbon oil; and removing the surplus oil, substantially as described. 10

In testimony whereof I affix my signature.

EUGENE P. SCHOCH.